

## UNITED STATES PATENT OFFICE.

CHARLES D. PARKS, OF DANBURY, CONNECTICUT.

## TREATED FUR AND ART OF TREATING THE SAME.

No Drawing.

Application filed June 30, 1923. Serial No. 648,850.

*To all whom it may concern:*

Be it known that I, CHARLES D. PARKS, a citizen of the United States, and a resident of Danbury, in the county of Fairfield, State of Connecticut, have invented an Improvement in Treated Fur and Art of Treating the Same, of which the following is a specification.

This invention relates to treated fur or similar material and to the art of treating the same and with regard to its more specific features to such material treated in preparation for the manufacture of felt therefrom.

One of the objects of the invention is to provide fur or the like having certain desired characteristics or properties in a high degree and free from certain objectionable characteristics often present in such material. Other objects are to provide material of the above nature especially adapted for the practical manufacture of felt and possessing certain qualities whereby efficient dyeing is facilitated and whereby a lower grade of raw material may be used. Another object is to provide material of the above nature capable of forming felt in a highly efficient and satisfactory manner and which is substantially free from harmful ingredients. Another object is to provide a practical and effective art of treating fur or material of a similar nature whereby the same may be prepared in a highly satisfactory manner for the manufacture of felt therefrom. Other objects will be in part obvious or in part pointed out hereinafter.

The invention accordingly consists in the features of composition, constitution of parts and in the several steps and relation and order of each of the same to one or more of the others thereof, all as will be illustratively described herein and the scope of the application of which will be indicated in the following claims.

As conducive to a clear understanding of the several features of this invention, it may be here noted that the subject matter of this invention deals primarily with material such as fur or similar fibrous animal products treated or prepared principally for the manufacture of felt therefrom, as for example for the manufacture of felt hats, and with the art of carrying on such treatment. Fur or similar material as it comes from the animal is ordinarily in its natural state not suitable for the manufacture of felt and when

it reaches the hands of the felt manufacturer, it has been subjected to a preparatory treatment adapted to bring out certain desired qualities for felting. The broad idea of such preliminary treatment or preparation is commonly known as carroting and the fur after such treatment is commonly known as carroted fur. The formation of felt from fur or the like is brought about by the individual fibres in contact with each other overlapping and interlocking and it is to increase this tendency of the fur to work together and interlock that the carroting process is resorted to. The natural fur has associated therewith a certain amount of oil or grease or gummy substance and other foreign material which for the sake of convenience and clarity will be hereinafter generally referred to as wax. Fur after proper carroting treatment should have such wax removed or rendered soluble and in such condition the fur has the properties which are most to be desired for proper and efficient felting. The surface of a fur or hair fibre, as is commonly known, is coated with a layer of overlying scales or barbs and the fur after having the wax rendered ineffective by the carroting treatment has these scales loosened or released to some extent and thus loosened or released the scales or barbs assist materially in the interlocking action of the fibres to form felt. It may be here noted that the term "fur having felting properties" is used broadly to indicate fur having such characteristics that when subjected to an ordinary felting process it will felt.

In the manufacture of felt, as for example in the manufacture of felt hats, the fur is continually handled throughout the different processes, many of the processes involving the application of hot water and steam and therefore a fur which in the carroting process has been impregnated with a poisonous material is extremely objectionable. The material commonly employed at the present time as a carroting substance is mercuric nitrate, prepared from nitric acid and mercury. Fur which has been treated with such a carroting material is, when it comes to the felt manufacturer, impregnated with a poisonous acid substance and the poisonous fumes which are released therefrom during the processes of felt manufacture are highly objectionable and unhealthful. In addition to

the objectionable poisonous character of fur treated with such material, the fur is apt to be roughened or partially disintegrated as a result of the strong acid treatment. The provision of treated furs or the like which are efficiently prepared to have the properties most desired for felting, which are free from poisonous ingredients and which are characterized by other advantageous qualities is among the dominant aims of this invention.

The carroting process of this invention is most conveniently carried out by brushing the carroting material into the fur in the form of a solution and in this manner the best results are obtained in that a solution may readily reach all the fibres of the fur and a regular, uniform treatment thereof may be had. This process of carroting the fur preferably comprises the application to the fur of a solution of a mixture of an oxidizing agent and an alkaline cleansing agent.

The preferred form of carroting substance employed in the carroting process of this invention comprises a solution of a mixture of a non-acid or hydroxide cleansing agent and an oxidizing agent. The cleansing agent is preferably hydroxide of sodium but other cleansing agents may be employed with good results, such as hydroxides of other elements of the alkali metal family, for example hydroxide of potassium. The oxidizing agent preferably employed is hydrogen peroxide. The mixture of the cleansing agent and the oxidizing agent in solution may be prepared in other ways, in so far as the broader features of this invention are concerned, but is preferably prepared from a peroxide of the element forming the hydroxide cleansing agent by mixing the peroxide with water. For example, peroxide of sodium is supplied commercially in the form of a yellowish white powder which is decomposed by water forming sodium hydroxide and hydrogen peroxide. Sodium hydroxide is an excellent cleansing agent having a corrosive action upon most animal and vegetable materials and hydrogen peroxide is a strong oxidizing agent. In forming such a solution, it is desirable to start with an ample volume of water and sift the peroxide slowly thereinto, stirring the mixture in order to keep the temperature down. The reaction of the peroxide with the water generates considerable heat and the temperature should be kept down to about 55° F. When the desired strength of the solution is obtained by thus gradually adding the sodium peroxide to the water, the solution is ready for application to the carroting process upon the fur or hair. The strengths of the solution preferably employed will be more fully set forth herein-after.

The process of applying the carroting material to the fur may be carried on while the

fur is still upon the skin or it may be carried on after the fur has been removed from the skin or pieces. The preferred method is to apply the carroting solution to the fur upon the skin. In accordance with this method, the solution is preferably applied to the fur by means of a brush, care being taken to thoroughly brush the material into the fur and evenly treat all parts thereof. The fur is then dried and is then ready for removal and other steps in the manufacture of felt. In the other method, namely that of applying the carroting material to the fur after it is removed from the skin or pieces, the process consists preferably of immersing the loose fur in the solution and then drying the fur. In the first mentioned method, namely that of brushing the solution into the fur on the skin, a much stronger solution of the carroting material is required than in the second method wherein the loose fur is immersed in the solution. When using the solution by brushing it into the fur on the skin, the strength of the solution may vary between the approximate limits of 1° Baumé and 10° Baumé. However, it is found that the best results are better assured if the strength of the solution is kept within the limits of about 2½° Baumé and 7° Baumé. The strength of solution to give the best results may, however, vary with the type and quality of the fur being carroted, it being found that with certain grades of fur a solution having a strength of about 6° Baumé gives the best results. To give a solution having a strength of about 6° Baumé, approximately 1 pond of sodium peroxide is dissolved in 3 gallons of water. If the strength of the solution is too high, the carroted fur will be injured and if the strength of the solution is too low, the full results desired of the process are not achieved. When treating loose fur, that is fur detached from the skin or pieces, it is found that the strength of the solution may vary approximately from 1 pound of sodium peroxide in 300 gallons of water up to 6 pounds in 300 gallons of water. In this latter method, however, the preferred proportions are about 2 pounds of sodium peroxide in 300 gallons of water, it being found that the solution resulting from such proportions gives good results when treating the fur after being detached from the skin. It seems probable that in the process of treating the loose fur, the carroting solution is afforded an opportunity of working inside the fur fibres through the clipped, chopped or cut ends which opportunity is not afforded in the process of treating the fur upon the skin and this may account for the relative weakness of solution needed for suitable carroting of the detached fur.

In the carroting process embodied in this

invention, as described above, the fur or other felting material has substantially all the wax or gummy substance removed therefrom by being made soluble and absorbent 5 of water and then washed out. The car-rotted fur is non-poisonous and non-acid having either an alkaline or neutral reaction. The non-poisonous character of the carotted fur renders it far more suitable for handling 10 and far more healthful from the standpoint of workmen who come into continual contact with the fur during the process of felt manufacture therefrom than is fur carotted by the usual nitrate of mercury process and 15 impregnated with the poisonous nitrate. The carrotting process of this invention is much less liable to harm the fur and detract from the life thereof than is an acid treatment. Furthermore, felt prepared from an 20 alkaline fur is far better suited for dyeing than is a fur impregnated with acid as it takes the dye much easier. In the process of dyeing fur or felt, the dye is first thoroughly and evenly applied to all parts there- 25 of, whereupon an acid is employed to set the dyes. In order to obtain the desired uniform results of dyeing, it is highly desir- able that the fur or felt be free from acid in order that premature setting of the dye may 30 be avoided and in order that an even and uniform application thereof may be had. It will readily be seen that an alkaline fur is particularly adapted for this purpose, not only on account of the absence of acid but 35 on account of its neutralizing effect on any acid that may be in the dyes. In addition the carrotting processes of this invention enable the dyer to obtain lighter shades in the dyed fur as the carrotting materials have a 40 bleaching or lightening action on the fur.

In the manufacture of felt hats and of other kinds of felt, it is common practice to mix with the good quality felting fur or fleece fur as it is called, a proportion of 45 cheaper fur which felts little, if at all, thus reducing the price of the fur required for a hat and in some respects improving the hat. The amount of this cheaper fur or 50 filler fur, as it is called, which can be em- ployed is, of course, limited. When the fleece fur, as well as the cheaper filler fur, is treated in accordance with the carrotting processes of this invention, it is found that 55 due to the superiority of the felting qualities attained, a much larger proportion of the filler fur may be employed than is pos- sible when the old acid process of carrotting is used.

From the above, it will be seen that there 60 is herein provided an art of preparing fur or similar material which attains many dis- tinct, practical and useful advantages and which is particularly well adapted for ap- plication to practical use. Furthermore, the 65 resulting product is one which embodies

many qualities greatly to be desired in such material.

As various possible embodiments might be made of the above invention and as the embodiments above set forth might be va- 70 ried and as the art herein described might be modified in various ways all without de- parting from the scope of the invention, it is to be understood that all matter herein set forth is to be interpreted as illustrative and 75 not in a limiting sense.

I claim as my invention:

1. The herein described art of preparing fur or the like for felting which consists in applying an alkaline solution of an oxidiz- 80 ing agent to the fur on the skin and adapted to give the fur felting properties, drying the fur, and removing the fibers from the skin.

2. Carrotted fur or the like having upon the fibers thereof a product resulting from 85 the reaction with the natural wax thereon of an aqueous solution of an oxidizing agent and a cleansing agent.

3. Carrotted fur or the like having upon the fibers thereof a product resulting from 90 the reaction with the natural wax thereon of a solution of a hydroxide of an alkali metal and an oxidizing agent.

4. Carrotted fur or the like having upon the fibers thereof a product resulting from 95 the reaction with the natural wax thereon of a solution of a hydroxide of an alkali metal and hydrogen peroxide.

5. Carrotted fur or the like having upon the fibers thereof a product resulting from 100 the reaction with the natural wax thereon of a solution of sodium peroxide dissolved in water.

6. The herein described art which con- 105 sists in treating fur fibers with a solution of an oxidizing agent and a cleansing agent and adapted to give the fur felting properties, drying the fur fibers, and felting the fibers together.

7. The herein described art which consists 110 in treating fur fibers with a solution of sodium peroxide dissolved in water and in proportions to give the fur felting properties, drying the fibers, and subjecting the fibers to felting action.

8. The herein described art of preparing fur or the like for felting which consists in treating the fur with a solution of an oxidizing agent and a cleansing agent and adapted to give the fur felting properties. 115

9. The herein described art of preparing fur or the like for felting which consists in treating the fur with a solution com- 120 prising a hydroxide of an alkali metal and an oxidizing agent in such proportions that the fur fibers are thereby given felting prop- 125 erties.

10. The herein described art of preparing fur or the like for felting which consists in treating the fur with an aqueous solution 130

- of a hydroxide of an alkali metal and hydrogen peroxide in such proportions that the fur fibers are thereby given felting properties.
11. The herein described art of preparing fur or the like for felting which consists in treating the fur with an aqueous solution of sodium hydroxide and hydrogen peroxide in such proportions that the fur fibers are thereby given felting properties.
12. The herein described art of preparing fur or the like for felting which consists in treating the fur with a solution of sodium peroxide in water having a strength between 1° Baumé and 10° Baumé.
13. Carroted fur or the like having upon the fibers thereof a product resulting from the reaction with the natural wax thereon of a aqueous solution of an oxidizing agent and a cleansing agent and comprising fibers removed from the skin.
14. Carroted fur or the like having upon the fibers thereof a product resulting from the reaction with the natural wax thereon of a solution of sodium peroxide dissolved in water and comprising fibers removed from the skin.
15. The herein described art of preparing fur or the like for felting which consists in treating the fur with a solution of sodium peroxide dissolved in water and in proportions to give the fur felting properties.
16. The herein described art of preparing fur or the like for felting which consists in treating the fur with a solution of sodium peroxide in water having a strength between 2½° Baumé and 7° Baumé.
17. The herein described art of preparing fur or the like for felting which consists in treating the fur with a solution of sodium peroxide and water in such proportions that the fur fibers are thereby given felting properties, and in thereupon drying the fur to retain on the fibers thereof the product of the reaction of the solution with the natural wax on the fibers.

In testimony whereof, I have signed my name to this specification this 19th day of June 1923.

CHARLES D. PARKS.